

## UNITED STATES PATENT OFFICE

2,257,601

## METHOD OF LUBRICATION

Frank W. Hall, New York, and Charles C. Towne,  
Beacon, N. Y., assignors to The Texas Com-  
pany, New York, N. Y., a corporation of Dela-  
ware

No Drawing. Application August 6, 1938,  
Serial No. 223,487

2 Claims. (Cl. 252—53)

This invention relates to a lubricating oil, and particularly to a motor oil adapted for lubrication of the bearings and cylinders of internal combustion engines, such as automotive engines, airplane engines, Diesel engines and the like.

One of the principal objects of the invention is to provide an improved lubricating oil of this type which is compounded with a small proportion of an additive material that is effective to reduce or inhibit bearing corrosion and lacquer formation, while affording other advantages as more fully set forth below.

In accordance with the present invention, there is added to a mineral lubricating oil of this type a small proportion of a phosphatide compound or phospholipin, such as lecithin. The phosphatides, or the lecithins as they are frequently called, belong to the class of compounds having the general formula



where R and R' are similar or dissimilar fatty acid radicals such as those derived from stearic, palmitic, oleic acids, etc., and where X represents an amino alcohol group. In the case of lecithin, X or the amino alcohol group is choline— $\text{CH}_2\text{CH}_2\text{N}(\text{CH}_3)_3\text{OH}$ ; and in the case of cephalin X is colamine— $\text{CH}_2\text{CH}_2\text{NH}_2$ . Other types of compounds falling within the class of phosphatides can be employed such as sphingomyelin. Also metal derivatives or salts of the lecithins can be employed. For example, the free acid group of the compound can be neutralized with alkali, alkaline earth and other bases to form the corresponding salts thereof.

A preferred composition for this purpose is commercial soybean lecithin, such as the product known commercially as "Lipoidol" which consists essentially of about equal proportions of lecithin and cephalin with a smaller proportion of soybean oil. In some cases it is found preferable to employ a bleached commercial soybean lecithin, such as the product sold commercially as "Colloidol BT" which is commercial soybean lecithin bleached with hydrogen peroxide and dibenzoyl peroxide, or the product sold commercially as "Colloidol HX" which is commercial soybean lecithin bleached with hydrogen peroxide. If desired, the commercial soybean lecithin can be purified by extracting the soybean oil with acetone to obtain a product consisting essentially of lecithin and cephalin, which is also suitable for the purposes of the present invention. Also, the cephalin constituent can be separated from the lecithin by alcohol extraction, and either the purified lecithin or purified cephalin or mixtures of the two in any desired

proportion may be employed for purposes of the present invention. However, it has been found that the purified constituents do not display any marked improvement over the commercial soybean lecithin, and the latter is generally preferred for economical reasons. Another suitable commercial product for purposes of this invention is "clearate" which is a phosphatide compound, as defined above.

10 Wherever the expression "phosphatide compound" is used throughout the description and claims, it is to be understood that this includes any of the purified compounds or derivatives thereof falling within this group, as well as any of the comparatively impure mixtures such as the commercial grades mentioned above.

In accordance with the present invention, the phosphatide compound is added to the motor oil in a critical proportion range of about 0.01—2.0%. It is found that these percentages are critical in securing the desired improvement with respect to inhibiting bearing corrosion and lacquer formation and without affecting other desirable properties of the oil, while proportions above this range produce undue sludging. In the case of motor oils adapted for automotive use, a range of 0.01 to 0.25% appears most satisfactory, with about 0.1% preferred. Somewhat higher percentages may be employed in Diesel lubricating oils or airplane oils where it is desired to improve materially the ring sticking properties of the oil in addition to obtaining the benefits of inhibiting bearing corrosion and lacquer formation. A very satisfactory method for adding the phosphatide compound to the mineral lubricating oil is to first form a concentrate, such as a 50% solution of the lecithin or other phosphatide compound in a S. A. E. 30 oil or other lubricating oil within the motor oil viscosity range, and then add the concentrate to the mineral lubricating oil in an amount sufficient to give the desired percentage of phosphatide compound therein.

The additive of the present invention is particularly effective in connection with highly solvent refined lubricating oils, such as the modern motor oils which have been refined with a solvent having high selectivity between naphthenic and paraffinic constituents of the oil, such as furfural, beta beta dichlor ethyl ether, nitrobenzene, phenol, cresylic acid, chlorphenol, and the like.

45 The modern development of internal combustion engines with extremely small clearances between piston and cylinder wall, together with the modern development of highly solvent refined lubricating oils for use in the crankcases of such engines, has given rise to the problem of so-called varnish or lacquer formation. This lacquer generally appears as a yellowish or reddish brown film which deposits upon the metal sur-

faces, piston rings and cylinder walls during operation of the engine over extended periods of time. In the newest engines having extremely small clearances and high compression, this problem is so severe as to frequently result in seizure of the pistons when the motor is stopped and allowed to cool.

Further, the modern development of the highly refined motor oils together with the modern development of the new type bearings including the connecting rod and main bearings, of internal combustion engines, which has involved a departure from the old Babbitt bearings and has given rise to new alloy bearings of the type of cadmium-silver, copper-lead, and the like, has also presented the industry with the problem of bearing corrosion. This latter problem has been recognized for the last several years, and various materials have been heretofore suggested as additives for lubricating oil to inhibit such bear-

properties unrelated to the fiber wetting or film action of the prior art.

As illustrative of the effectiveness of the phosphatice compounds of the present invention in reducing bearing corrosion, the following test was used. A bushing lined with the same cadmium-silver or other alloy as employed in connecting rod bearings in some automotive engines, was immersed in a pot of the oil to be tested, the oil being heated to a temperature of the order of 325-350° F. The oil is circulated between the bushing and its journal by a suitable propeller or "whirligig" for a period of five hours. The bushing is removed from the pot at intervals of five hours, weighed and returned. The loss in weight is expressed in milligrams and is considered the corrosion loss. The reference oil employed in these tests was a furfural refined dewaxed Mid-Continent lubricating oil of S. A. E. 30 grade.

| Test oil                                | Percent substance added | 2½ hr. | 5 hr. | 10 hr. | 15 hr.   | 20 hr.   | 25 hr. | 30 hr. | 35 hr. | 40 hr. |
|-----------------------------------------|-------------------------|--------|-------|--------|----------|----------|--------|--------|--------|--------|
| Reference oil                           | 100% blank              | 1      | 3, 1  | 34, 39 | 212, 236 | 473, 456 | 4      | 5      | 5      | 5      |
| +Clearate BB                            | 0.25                    | 0      | 1     | 0      | 0        | 4        |        |        |        | 6      |
| +Clearate BB with soya bean oil removed | 0.25                    |        | 1     | 1      | 2        | 3        | 4      | 5      | 9      | 9      |
| +Cephalin from Clearate                 | 0.25                    |        | 1     | 2      | 4        | 6        | 7      | 8      | 10     |        |
| +Lecithin from Clearate                 | 0.25                    |        | 2     | 3      | 4        | 5        | 5      | 6      | 8      | 9      |
| +Crude Lecithin                         | 0.25                    |        | 1     | 3      | 4        | 5        | 5      | 6      | 8      | 7      |
| +Coloidol BT                            | 0.1                     |        | 2     | 3      | 3        | 4        | 5      | 5      | 6      | 6      |
| +Lipoidol                               | 0.1                     |        | 5     | 8      | 10       | 11       | 11     | 11     | 14     | 20     |

ing corrosion. However, the materials heretofore suggested and used for this purpose, such as triphenyl phosphite, are ineffective in overcoming the more recent problem of lacquer formation. The phosphatide compound of this invention is unique in combining in one substance the properties of preventing or minimizing this objectionable lacquer formation and of also inhibiting bearing corrosion, reducing cylinder and piston wear, and improving ring sticking of the motor oil to which the compound is added in the small proportion range specified above.

We are aware that it has been heretofore suggested to add lecithin together with a soap to a light lubricating oil having a Saybolt viscosity of less than 100 seconds at 100° F. to produce a textile fiber spraying oil (see U. S. Patent No. 2,002,885). The lecithin was employed here to improve the wetting or filming character of the oil for the textile fibers. The present invention is distinguished in the addition of lecithin to a different type of lubricating oil (a motor oil adapted for lubricating the bearings and cylinders of an internal combustion engine) which is of a different viscosity range as falling within the motor oil viscosity range and having a Saybolt viscosity in excess of 100 at 100° F. and generally in excess of 150 at 100° F. By motor oil viscosity range is understood that range embracing the motor oils falling within the S. A. E. 10 to 60 range as well as certain heavier motor oils adapted for special use in heavy duty truck or bus engines at higher atmospheric temperatures, and having a viscosity range varying from about 90 seconds at 130° F. up to about 150 seconds at 210° F. Saybolt Universal, as shown on page 444 of the 1936 edition of the S. A. E. Handbook. The present invention is also distinguished from the above mentioned patent in that the additive is employed for an entirely different purpose of inhibiting lacquer formation and bearing corrosion in addition to the other advantages enumerated, which are entirely new and unexpected

From the above tests, it is noted that in the case of the reference oil there is a short induction period of less than ten hours within which little corrosion takes place, but then the rate of corrosion increases rapidly for the duration of the run up to twenty hours. However, in the case of the reference oil blended with the phosphatide compounds specified, it was noted that very little corrosion took place over the entire period of the run which was extended to forty hours.

The lacquer formation test thus far developed is primarily a qualitative one. This may be carried out by employing the oil in an engine having extremely small clearances of the order of 5/10,000 to 7/10,000 of an inch and running the engine for an extended period of time with frequent stopping and cooling to test for piston seizure, and finally inspection of the piston and cylinder wall after the termination of the test. In the case of the reference oil, a furfural refined dewaxed Mid-Continent distillate of S. A. E. 30 grade, piston seizure may occur frequently after a run of comparatively short duration; and inspection of the parts will show the presence of an appreciable lacquer film. On the other hand, similar runs conducted with the reference oil compounded with about 0.1-0.25% of the phosphatide compounds specified above may be carried out satisfactorily without piston seizure, and inspection will show the metal surfaces of the piston and cylinder wall to be comparatively free of any lacquer film.

Without wishing to be bound to any particular theory, it is believed that the phosphatides possess an adsorption action in preventing lacquer formation. Apparently such phosphatide compounds form a colloidal solution or colloidal suspension with lubricating oil which is extremely stable. For example, when a lubricating oil containing lecithin within the proportion range set out above is heated and oxidized at 350° F. for eight hours in the Indiana oxidation test, the

lecithin does not settle out but remains in effective colloidal solution or suspension. Other previously known bearing corrosion inhibitors, such as triphenyl phosphite, partially separate from the oil under this test. This colloidal solution or suspension of lecithin is believed to provide a multitude of surfaces within the oil upon which the lacquer particles are adsorbed as they are formed, and are thereby prevented from plating out on the metal parts of the piston and cylinder wall. The fact that the colloidal solution or suspension so formed is not separated by filtration through the standard types of oil filters employed in automotive engines, after the compounded oil has been in engine service, shows that the lecithin or other phosphatide compound remains operative and effective in an internal combustion engine over extended periods of time, so that its anti-corrosive and anti-lacquer forming properties are retained. Moreover, the lecithin functions to maintain a finer dispersion of such sludge as may be formed in the oil during engine operation.

Typical results on the Indiana oxidation test on the reference oil (a furfural refined dewaxed Mid-Continent distillate of S. A. E. 30 grade) and on the reference oil compounded with the noted percentages of the phosphatide compounds are set forth in the following table:

Blank oil, furfural refined dewaxed Mid-Continent distillate of S. A. E. 30 grade

| Material added                         |           | Clearate  | Clearate with soya bean oil removed | Cephalin from Clearate | Lecithin from Clearate | Crude lecithin |
|----------------------------------------|-----------|-----------|-------------------------------------|------------------------|------------------------|----------------|
| Cone. percent.....                     |           | 0.25      | 0.25                                | 0.25                   | 0.25                   | 0.25           |
| Original sample vis. S. U. 210° F..... | 63-63     | 63-63     | 62                                  | 63                     | 62                     | 62             |
| Neut. No.....                          | 0.01-0.01 | 0.07-0.08 | 0.04-0.04                           | 0.04-0.04              | 0.04-0.04              | 0.03-0.03      |
| Sap. No.....                           | <0.5      | <0.5      | 0.7-0.7                             | 0.06-0.06              | <0.5                   | 0.8-0.6        |
| Indiana oxidation test:                |           |           |                                     |                        |                        |                |
| 10 mg. point.....                      | 74        | 18        | 10                                  | 20                     | 82                     | 74             |
| 100 mg. point.....                     | 126       | 128       | 130                                 | 142                    | 142                    | 138            |

The above tests show that the addition of the phosphatide compound may reduce the time required to reach the ten milligram point, but in every case the time required to reach the 100 milligram point of sludge is increased, thus indicating that the phosphatide is also effective to reduce oxidation or sludging as determined by the Indiana oxidation test over an extended period of time. The reduction in the time to reach the ten milligram point is attributable to the sludging characteristics of the phosphatide compound or lecithin itself, and apparently is not due to any effect that the additive has upon the initial sludging characteristics of the lubricating oil. Moreover, most of this sludge so formed from the lecithin is of the colloidal type mentioned which is believed valuable in promoting the inhibiting of lacquer formation as discussed above.

Another problem which has more recently come to the fore, particularly in the case of Diesel engines such as those employed in tractors, is that of a sludge deposit in the compression ring grooves and in the oil ring slots of the piston and piston rings. It is found that these deposits may accumulate to such an extent as to cause stuck rings and scoring of the cylinder wall. The phosphatide compounds of the present in-

vention are also effective in reducing this oil ring sludge deposit, as is evident from the following runs made on an SO<sub>2</sub> refined pale lubricating oil having a viscosity of 750 and 100° F., and on the same oil compounded with 1.0% of Lipoidol. In this test, a single cylinder C. F. R. Diesel engine is employed, which is run for thirty-six hours at 1200 R. P. M. at 210° F. jacket temperature with an artificially enriched fuel mixture and a fuel rate of 26 cc. per minute. After the run, the engine is taken down, the dirty piston rings are weighed, then the rings are cleaned by washing in benzol, and the cleaned and dried rings again weighed. This gives the total deposit including solid material and oil in the oil ring slots. The benzol is then evaporated to dryness, and the solid material taken up in 86° naphtha to dissolve out the oil. The naphtha is then distilled off and the oil weighed. The difference in weight between the total weight of the oil ring deposit and the weight of the oil is expressed as milligrams of oil-free deposit in the oil rings. The compression ring grooves are also cleaned in a similar manner and the weight of oil-free deposit in these grooves determined. Likewise, the amount of 86° naphtha insoluble sludge in the crank case oil is also determined.

The following is an example of typical results obtained in this test:

|                                  | Mg. oil-free deposit in compression ring grooves | Mg. oil-free deposit in oil rings | Mg. 86° naphtha insoluble sludge in crankcase oil |
|----------------------------------|--------------------------------------------------|-----------------------------------|---------------------------------------------------|
| Reference oil                    | 450                                              | 323                               | 76                                                |
| Reference oil plus 1.0% Lipoidol | 321                                              | 129                               | 54                                                |

The phosphatide compounds of the present invention are also effective in reducing engine wear, as determined in the so-called "low temperature wear test." This test is carried out on a C. F. R. single cylinder engine operating with a jacket temperature of 80° F. Before the test, the engine is taken down, and the piston rings are carefully cleaned and weighed. The engine is then assembled, operated for twenty hours at 900 R. P. M. with 1° spark advance and wide open throttle, and again taken down and rings cleaned and weighed. This difference in weight of the rings before and after the twenty hours of operation is computed as milligrams of ring wear.

The following results were obtained in this test on an acid treated and clay contacted Mid-Continent distillate of S. A. E. 20 grade, and on

this reference oil compounded with 1% of Lipoidol:

| Oil tested                                             | Ring wear |
|--------------------------------------------------------|-----------|
| Reference oil (average of two runs)                    | 259       |
| Reference oil plus 1.0% Lipoidol (average of two runs) | 176       |

The above test shows a 32% improvement of the compounded oil over the base oil. The phosphatide compounds of the present invention are also effective in reducing ring sticking of a motor oil. To illustrate this effect, a test is employed using a C. F. R. single cylinder engine operating at 900 R. P. M. with a 5:1 compression ratio, with 1° spark advance and wide open throttle, the jacket temperature being maintained at 375° F. The engine is equipped with a cast iron solid skirt piston with conventional piston rings. In preparing the engine for testing, the crank case, cylinder and piston are first cleaned thoroughly to remove all deposits and to provide a perfectly clean engine. The engine is then reassembled and the crankcase charged with the required amount of oil, generally 3000 c. c. The engine is then operated to give maximum power under the conditions set forth above for an interval of time, generally eighteen hours. The oil is then drained immediately after stopping, the

was required in the initial run on this oil. It is assumed that this means that engine conditions are changing over the period of the three runs. For purposes of calculation, it is assumed that 5 engine conditions which affect ring sticking change uniformly with running time over the three runs considered. The average sticking time for the reference oil is therefore not taken as the mean of the two reference runs, but is interpolated for the time at which sticking occurs with the test oil. The actual time required to stick the rings with the test oil is then compared with this interpolated or bracketed 15 average time for the reference runs and expressed as the per cent the test oil is better or worse than the reference oil with respect to the time required to stick rings.

In a test of this type on a typical airplane oil and on this oil compounded with 1.0% of Lipoidol, the compounded oil showed a 125% improvement over the reference oil.

In addition to the advantages enumerated above, it is found that these phosphatide compounds and particularly the purified compounds or the bleached commercial soybean lecithin can be added to high grade typical motor oils without objectionably affecting desirable properties or tests of these oils, as illustrated in the following table:

|                         | Oil used                                                                    |               |               |
|-------------------------|-----------------------------------------------------------------------------|---------------|---------------|
|                         | Blank oil (fur-fural refined de-waxed Mid-Cont. dist. of S. A. E. 30 grade) | Same ref. oil | Same ref. oil |
| Material tested         |                                                                             | Clearate      | Colloidol BT. |
| Percent material        |                                                                             | 0.25          | 0.1           |
| Gravity, °A. P. I.      | 28.2, 28.2                                                                  | 28.1, 28.1    | 28.1, 28.1    |
| Flash, C. O. C. °F.     | 460                                                                         | 460           | 460           |
| Fire, C. O. C. °F.      | 530                                                                         | 530           | 525           |
| Viscosity:              |                                                                             |               |               |
| 100° F., S. U.          | 510-511                                                                     | 512-513       | 512-511       |
| 130° F., S. U.          | 62-62                                                                       | 62-62         | 62-5-63       |
| 210° F., S. U.          | 87                                                                          | 87            | 92            |
| Vls. index              | 255-6"                                                                      | 285-6"        | 270-6"        |
| Color—Lovibond          |                                                                             |               |               |
| Pour, °F.               | 0                                                                           | 0             | +5° F.        |
| Carbon residue, percent | 0.11-0.10                                                                   | 0.11-0.11     | 0.12-0.13     |
| Neut. No.               | 0.01-0.01                                                                   | 0.08-0.08     | 0.03-0.03     |
| Sap. No.                | <0.5                                                                        | <0.5          | <0.5          |
| Cloud                   | +6,+6                                                                       | +6            | +6° F.        |
| Ash, percent            | Trace                                                                       | 0.02          | Trace         |

engine allowed to cool for at least three hours 50 and then the cylinder removed and the piston rings inspected. If, upon inspection, the rings are found free, the cylinder and oil are replaced and the run continued for an additional eighteen hours, when it is again disassembled in the man- 55 ner set out above and the rings reinspected. This procedure is continued until sticking occurs, generally of the top piston ring, or until the run has continued for such a length of time without actual sticking. If, at any inspection, rings are 60 on the verge of sticking, the additional run may be reduced to twelve hours or less. If any severe ring sticking condition is observed, the sticking time is estimated at some value between that of the final and the preceding inspection. 65 An accuracy of plus or minus six hours is generally obtained. No make-up oil is added to the crankcase during a complete run on any oil, as this is found to reduce the accuracy of the run.

Three runs are required to rate an oil being 70 tested in comparison with a reference oil. The reference oil is run both before and after the test sample. It is often found that a substantially different time to attain stuck rings is required in the final run on the reference oil than 75

Obviously, many modifications and variations of the invention herein set forth may be made without departing from the spirit and scope thereof, and therefore only such limitations should be imposed as are indicated in the appended claims.

We claim:

1. The method of lubricating connecting rod and main bearings of the new alloy type and cylinders and pistons of an internal combustion engine, which comprises maintaining between the bearing surfaces and on the cylinder and piston walls films of a mineral lubricating oil which provide an effective lubricating action but which normally tend to corrode the said alloy bearings and to produce varnish deposits on the said cylinder and piston walls, and minimizing the said bearing corrosion and varnish deposits while maintaining the effectiveness of the lubricating action by incorporating in the said mineral lubricating oil about 0.01-2.0% of a phosphatide compound.

2. The method according to claim 1, in which the phosphatide compound is lecithin.

CHARLES C. TOWNE.  
FRANK W. HALL.